

## [54] HEAT TREATMENT FOR WROUGHT ZINC-ALUMINUM ALLOYS

[75] Inventors: **Edouard Gervais**, Montreal; **Pierre Chollet**, Pierrefonds, Quebec, both of Canada

[73] Assignee: **Noranda Mines Limited**, Toronto, Canada

[22] Filed: May 5, 1972

[21] Appl. No.: 250,556

## [30] Foreign Application Priority Data

July 21, 1971 Canada ..... 118721

[52] U.S. Cl. .... 148/11.5 R, 148/13

[51] Int. Cl. .... C22f 1/16

[58] Field of Search ..... 148/11.5 R, 13

[56]

## References Cited

## UNITED STATES PATENTS

3,676,115 7/1972 Hare et al..... 75/178 AM

Primary Examiner—W. Stallard

[57]

## ABSTRACT

The creep resistance and strength of wrought zinc-aluminum alloys having a zinc-aluminum eutectoid transformation is improved by a heat treatment comprising slow cooling the alloy from a temperature between its eutectoid and solidus temperatures to below its eutectoid temperature and subsequently rapidly cooling the alloy.

14 Claims, 3 Drawing Figures



PATENTED JAN 28 1975

3,862,863

SHEET 1 OF 3



FIG. I. TIME IN HOURS



FIG. 2.

PATENTED JAN 28 1975

3,862,863

SHEET 3 OF 3



FIG. 3

## HEAT TREATMENT FOR WROUGHT ZINC-ALUMINUM ALLOYS

This invention relates generally to a heat treatment for wrought zinc-aluminum alloys.

More particularly, the present invention is a heat treatment for wrought zinc-aluminum alloys having a eutectoid transformation, which optionally contain copper, magnesium, or bismuth to improve the creep resistance and the ultimate tensile strength of the alloys.

The heat treatment of the present invention is especially applicable to zinc-aluminum alloys containing about 12% to about 30% (preferably about 18% to about 30%) aluminum, 0% to about 10% copper, 0% to about 1% magnesium, 0% to about 3% bismuth and the balance zinc except for incidental impurities.

Considerable research has been conducted on zinc-aluminum alloys of near eutectoid composition since it is acknowledged that such alloys have a variety of commercial applications. In the applicants' U.S. Pat. application Ser. No. 108,199 filed Jan. 20, 1971, a heat treatment is disclosed for wrought zinc-aluminum alloys containing 18 to 30% aluminum, up to 3% copper, up to 0.1% magnesium, up to 0.1% lithium and the balance zinc apart from incidental impurities, wherein the physical properties of the alloy are improved by slow cooling the alloy to ambient or room temperature from a temperature above the eutectoid temperature and below the solidus temperature. A preferred embodiment of that invention involves slow cooling the alloy from about 380°C. to room temperature.

Difficulties with zinc-aluminum alloys have often been encountered due to the high creep rates of such alloys. A principal advantage of the heat treatment of the present invention is that the creep resistance of such alloys is improved as compared to alloys heat treated according to the method described by the same inventors in U.S. Pat. application Ser. No. 108,199.

A further advantage is that alloys heat treated according to the present invention have a higher ultimate tensile strength and hardness than alloys heat treated according to the method described in U.S. Pat. application Ser. No. 108,199.

The heat treatment according to the present invention comprises homogenizing and slow cooling wrought zinc-aluminum alloys having a zinc-aluminum eutectoid transformation from above the eutectoid temperature and below the solidus or eutectic temperature to a temperature below the eutectoid temperature where eutectoid decomposition is substantially complete, and then rapidly cooling the alloy to room temperature. By interrupting the slow cooling heat treatment process described in U.S. Pat. application Ser. No. 108,199 at a temperature of about 250°C. and then rapidly air cooling the alloy to room temperature, considerable improvement in the creep resistant properties is achieved as compared to an alloy which is slow cooled by furnace cooling to room temperature.

With reference to the preferred ranges of alloying constituents contemplated for treatment by the present invention it should be noted that the present heat treatment for a wrought zinc-aluminum alloy containing 12 to 30% aluminum, 0 to 10% copper, 0 to 1% magnesium, 0 to 3% bismuth, the balance being zinc except for incidental impurities comprises the steps of homogenizing and slow cooling the alloy from above its eutec-

toid temperature and below its solidus or eutectic temperature to a temperature below its eutectoid temperature whereat the eutectoid transformation is substantially complete, and rapidly cooling the alloy. The heat treatment according to the present invention also results in an increase in hardness and ultimate tensile strength as compared with alloys of the same composition slow cooled to room temperature. However, as will be seen from the data in the tables at the end of this disclosure, the improvement in creep resistance is a more significant feature of the present invention.

FIG. 1 is a series of cooling curves from 380°C. for a zinc-aluminum alloy.

FIG. 2 is a creep deformation curve for a typical zinc-aluminum alloy.

FIG. 3 is a graph showing the effect of copper content and magnesium additions on the ultimate tensile strength of zinc — 25% aluminum alloys heat treated according to the present invention and according to the method described in U.S. Pat. application Ser. No. 108,199.

According to the present invention, a heat treatment is provided for wrought zinc-aluminum alloys having a zinc-aluminum eutectoid transformation involving slow cooling the alloy from a temperature above its eutectoid temperature and below its solidus temperature to a temperature below the eutectoid temperature whereat the eutectoid transformation is substantially complete, and thereafter rapidly cooling said alloy.

The alloys investigated were produced by melting the elements in the desired proportions in an induction furnace and by semi-continuous casting using the controlled cooling method. The cast billets were extruded under lubrication at a temperature of 250°C. and the extrusion product was then cold drawn.

The heat treatment procedure consisted of two stages:

STAGE I - The alloy was slow cooled from a temperature above the eutectoid temperature and below the solidus or eutectic temperature after a brief period of homogenization. The homogenization temperature was the same temperature from which slow cooling is intended to commence. The average rate of cooling was preferably less than about 2.0°C./min. (For alloys with less than about 18% aluminum the solidus temperature becomes the eutectic temperature).

STAGE II- The slow cooling process of Stage I was interrupted below the eutectoid temperature, where eutectoid decomposition is substantially completed, and the sample was rapidly cooled, usually in air.

In FIG. 1, Curve 2 shows the cooling rate of a sample within the range described in the above-mentioned United States patent application. The other curves represent various cooling rates which were used during the study. The plateau shown on the curves corresponds to the eutectoid transformation; the eutectoid transformation starts at the beginning of the temperature arrest and is largely completed when the temperature decreases again. For the heat treatment to be fully effective, the sample should not be removed from the furnace before the end of the plateau.

An example of a cooling curve of Stage II according to the present invention is shown in FIG. 1 by the dotted line identified as Curve 2A. Curve 2A schemati-

cally represents air cooling from 250°C. to room temperature.

Stage I of the two heat treatments is the same; for example, the specimens are slowly cooled from about 380° to about 250°C. The improvement according to the present invention results from Stage II.

The exothermic eutectoid transformation results in a plateau of flattening of the cooling curve. The resumption of a normal cooling rate indicates that eutectoid transformation is substantially complete.

The tensile tests were carried out on a Tinius-Olsen tensile machine using 0.375 inch diameter samples at a cross head separation rate of 0.25 in./min. The percent elongation was determined over a 2 inch gauge length and the percent area reduction was determined from the minimum diameter of the sample at rupture.

The hardness of each sample was determined with a Vickers Hardness Tester; all measurements were made using a 5-kilogram load.

The creep test samples were designed in accordance with ASTM specification E.139-58T. All creep tests were carried out under a constant load of 20,000 lb/in.<sup>2</sup> and at a temperature of 68° ± 1°F.; the sample deformation over the two inch gauge length was recorded using an optical system. FIG. 2 shows a typical creep curve and defines the two criteria used to quantify the results. The first criterion corresponds to the well known inverse creep rate which is defined as the inverse of the slope of the straight portion (second stage creep); the units are day/%. The second criterion corresponds to the time required to reach 1% plastic deformation.

Table I shows the effect of various heat treating procedures on the mechanical properties of a zinc base alloy containing 25% Al, 1% Cu and 0.05% Mg.

A comparison of Examples 1 and 2 shows that a sample which is furnace cooled from 380°C. has greatly improved creep resistance (78 days/%) compared to a sample in the "as extruded and drawn" stage (2.5 days/%). The sample slow cooled from 380°C. shows lower tensile properties and hardness.

A comparison between Examples 2 and 3 illustrates that a sample that has been slow cooled from 380°C. to 250°C. and then air cooled shows a further improvement in creep resistance (266 days/%) compared to a sample which has been slow cooled from 380°C. without any interruption in the slow cooling. Example 3 with the interrupted cooling also shows some improvement in ultimate tensile strength and hardness over slow cooled Example 2.

Example 4 shows slow cooling from 290°C. where the improvement in creep resistance (3.6 days/%) compared to untreated Example 1 is only slight.

Example 5 shows slow cooling from 290°C. to 225°C. followed by air cooling and a further improvement in creep resistance (17.9 days/%) compared to slow cooled Example 4.

The effect on mechanical properties of heating (aging) the alloy for 3 hours at 250°C. followed by air cooling (Example 6) has been added to Table I to demonstrate that it is important to go above the eutectoid temperature. Hence, simply heating a sample to 250°C. and air cooling is not sufficient to develop a creep resistance comparable to those obtained when using the method of heat treating of the present invention.

From an examination and comparison of the Examples in Table I it is seen that the most improvement in

creep resistance is obtained by slow cooling the alloy from near the solidus temperature to a temperature below the eutectoid temperature and then rapidly cooling the alloy to room temperature.

5 Although the examples of the present application are limited to tests conducted by cooling from 380°C. and 290°C. respectively, slow cooling from any temperature between the eutectoid temperature and the solidus temperature would produce satisfactory results. In the 10 commercial use of the present invention slow cooling of the alloy should commence at a temperature that is sufficiently below the solidus temperature such that the solidus temperature would not accidentally be exceeded. Therefore, slow cooling from a temperature 15 that is safely below the solidus temperature and above the eutectoid temperature would comprise the temperature range for use in the present invention.

Tests were undertaken to determine the effect of the air cooling temperature (Stage II) on the mechanical 20 properties of a zinc alloy containing 25% Al, 1% Cu, 0.05% Mg which was first homogenized and slow cooled from either 380°C. or 290°C. Table II illustrates the results for samples slowly cooled from 380°C. to various temperatures at which rapid cooling 25 commences and compares them with the results obtained from the air cooling to room temperature from 380°C. The data demonstrates the importance of waiting until the sample has undergone complete eutectoid transformation before air cooling is commenced if high creep 30 resistance is to be obtained.

Table II further demonstrates that if the temperature at which air cooling starts is too low a loss in creep 35 resistance results. This table also shows that air cooling samples from temperatures below the eutectoid temperature gives superior hardness, creep and tensile strength properties than for a sample slowly cooled to room temperature.

Since the heat treatment consists of two stages, the 40 sensitivity to the cooling rate of each stage was investigated to determine the effect on the mechanical properties.

Table III demonstrates the effect of the average cooling 45 rate to 250°C. on the mechanical properties of alloys slowly cooled from 380°C to 250°C. (Stage I) and thereafter air cooled to room temperature (Stage II). It shows that the alloys and heat treatment are quite insensitive to a cooling rate of Stage I within the range shown in Table III; the only significant property variation is an increase in ultimate tensile strength and hardness obtained with the fastest cooling rate.

Heating treating with cooling from 290°C. is more 50 sensitive to cooling rate. Table IV shows that the slower cooling rate to a temperature of 225°C., although leading to a slight reduction of the ultimate tensile strength results in a significant increase of the creep resistance.

The effect of the cooling rate during the second stage 55 of the heat treatment is shown in Table V from which it is apparent that the faster the cooling, the higher the ultimate tensile strength, and the lower the tensile ductility. In view of the practical considerations, air cooling is preferred for most applications of the present invention.

Since the dimensional and structural stability of the 60 zinc-aluminum alloys is frequency of concern, tests were conducted to determine the performance of the material upon dry ageing. The test consists of heating the samples for 10 days at 95°C. Ten days exposure at

95°C. is considered the equivalent of ten years exposure at ambient temperature in regard to ageing stability according to the brochure entitled "ILZRO 12: A New Zinc Gravity Cast Alloy" published by the International Lead-Zinc Research Organization Inc., New York, April 1966.

Table VI illustrates the tensile properties before and after dry ageing at 95°C. for a zinc base 25% Al, 1% Cu, 0.05% Mg alloy heat treated according to the present invention. It demonstrates that the alloy was stable after heat treatment and that ageing only slightly reduced the ultimate tensile strength. The dimensional stability of the heat treated alloy was considered excellent.

FIG. 3 and Table VII demonstrate the wide range of alloys to which the present invention is applicable and also illustrate the effect that varying amounts of the different elements have on their tensile properties. In Table VII, the properties of alloys slowly cooled from 380°C. with and without rapid cooling from 250°C. are compared. FIG. 3 further demonstrates the advantages of the two-stage heat treatment over slow cooling from 380°C. to room temperature. It also shows, for both methods of heat treating, that the ultimate tensile strength increases with the copper content. Table VII shows that ductility decreases with increasing copper content. The alloys containing bismuth should preferably contain magnesium in the proportions described in our copending U.S. application Ser. No. 250,557. Table VII shows that the heat treatment of the present

invention is effective over the whole range of components investigated.

In addition to the heat treatment having a beneficial effect on alloys containing about 12% to about 30% aluminum, up to 10% copper, up to 1% magnesium, and up to 3% bismuth and the balance zinc it is anticipated that the heat treatment of the present invention should also have useful application for zinc-aluminum alloys which have a eutectoid phase transformation but which are outside the above range of compositions such as alloys containing 10 to 50% aluminum, and possibly alloys containing up to 15% copper.

It is preferable that homogenization take place at a temperature where the alloy is substantially all in the  $\alpha'$  phase, where it is possible to do so.

It can be appreciated from the foregoing that in its broad aspects the present invention involves a heat treatment for a wrought zinc-aluminum alloy having a zinc-aluminum eutectoid transformation comprising the steps of slow cooling the alloy from above its eutectoid temperature and below its solidus or eutectic temperature to a temperature below the eutectoid temperature whereat the eutectoid transformation is substantially complete, and subsequently rapidly cooling said alloy.

Generally, it can be readily seen that the present invention represents a significant advance in the art which should provide advantages and benefits to those segments of industry involved in the manufacture or use of the alloys which may be treated according to the present invention.

TABLE I

| Example | Metallurgical Condition                                                                             | Tensile Properties                                |              |                     |                                 | Creep Tests at 20,000 lb./in. <sup>2</sup> at 68°F     |                                        |
|---------|-----------------------------------------------------------------------------------------------------|---------------------------------------------------|--------------|---------------------|---------------------------------|--------------------------------------------------------|----------------------------------------|
|         |                                                                                                     | Ultimate Tensile Strength, (lb/in. <sup>2</sup> ) | % Elongation | % Reduction of Area | Hardness V.H.N. 5-Kilogram Load | Inverse Creep Rate $\pm$ 95% Confidence Limit (days/%) | Time to 1% Plastic Deformation, (days) |
| 1       | As extruded and drawn                                                                               | 62,600                                            | 29           | 70                  | 139                             | 2.6 $\pm$ 0.1                                          | 1.7                                    |
| 2       | Furnace cooled from 380°C (Curve 2 - FIG. 1 of United States Patent Application Serial No. 250,557) | 45,800                                            | 23           | 50                  | 107                             | 78 $\pm$ 6                                             | 53                                     |
| 3       | Furnace cooled from 380°C to 250°C (Curve 2) then air cooled                                        | 54,800                                            | 20           | 40                  | 124                             | 226 $\pm$ 12                                           | 150                                    |
| 4       | Furnace cooled from 290°C. Ref. United States Patent Application Serial No. 250,557                 | 45,100                                            | 32           | 58                  | 105                             | 3.6 $\pm$ 0.2                                          | 1.8                                    |
| 5       | Furnace cooled from 290°C to 225°C then air cooled                                                  | 50,200                                            | 31           | 55                  | 112                             | 17.9 $\pm$ 1                                           | 8.7                                    |
| 6       | 3 hours at 250°C and air cooled                                                                     | 55,200                                            | 25           | 57                  | N.A.                            | 12.5 $\pm$ 0.8                                         | 6.7                                    |

TABLE II

EFFECT OF AIR COOLING TEMPERATURE ON THE MECHANICAL PROPERTIES UPON SLOW COOLING FROM 380°C

| Stage II Air Cooling Temperature, °C | Tensile Properties                                |              |                     | Creep Tests at 20,000 lb./in. <sup>2</sup> at 68°F |                                                        |                                       |
|--------------------------------------|---------------------------------------------------|--------------|---------------------|----------------------------------------------------|--------------------------------------------------------|---------------------------------------|
|                                      | Ultimate Tensile Strength, (lb/in. <sup>2</sup> ) | % Elongation | % Reduction of Area | Hardness V.H.N. 5-Kilogram Load                    | Inverse Creep Rate $\pm$ 95% Confidence Limit (days/%) | Time to 1% Plastic Deformation (days) |
| 380                                  | 64,600                                            | 17           | 40                  | 143                                                | 45.8 $\pm$ 6.0                                         | 33                                    |
| Beginning of plateau                 | 68,900                                            | —            | 50                  | 158                                                | 37 $\pm$ 2                                             | 27                                    |
| End of plateau                       | 61,900                                            | —            | —                   | —                                                  | 88 $\pm$ 5                                             | 53                                    |
| 260                                  | 58,050                                            | 16           | 25                  | —                                                  | 162 $\pm$ 10                                           | 82                                    |
| 250                                  | 54,800                                            | 20           | 40                  | 124                                                | 226 $\pm$ 12                                           | 150                                   |
| 225                                  | 51,950                                            | 23           | 47                  | 120                                                | N.A.                                                   | N.A.                                  |
| 200                                  | 48,800                                            | 24           | 50                  | 113                                                | 119 $\pm$ 9                                            | 91                                    |
| 175                                  | 47,100                                            | 24           | 54                  | 107                                                | N.A.                                                   | N.A.                                  |
| 150                                  | 46,100                                            | 24           | 52                  | 107                                                | 85 $\pm$ 6                                             | 62                                    |
| 120                                  | 45,900                                            | 25           | 52                  | 104                                                | N.A.                                                   | N.A.                                  |
| 25                                   | 45,800                                            | 23           | 50                  | 107                                                | 78 $\pm$ 6                                             | 53                                    |

TABLE III

| Average Cooling Rate from 380 to 250°C, (°C/min.) | Tensile Properties                                |              |                     |                                 | Creep Tests at 20,000 lb/in. <sup>2</sup> at 68°F  |                                       |  |
|---------------------------------------------------|---------------------------------------------------|--------------|---------------------|---------------------------------|----------------------------------------------------|---------------------------------------|--|
|                                                   | Ultimate Tensile Strength (lb./in. <sup>2</sup> ) | % Elongation | % Reduction of Area | Hardness V.H.N. 5-Kilogram Load | Inverse Creep Rate ± 95% Confidence Limit (days/%) | Time to 1% Plastic Deformation (days) |  |
| Curve 1 1.8                                       | 58,700                                            | 16           | 40                  | 134                             | 210 ± 8                                            | 168                                   |  |
| Curve 2 1.01                                      | 54,800                                            | 20           | 40                  | 124                             | 226 ± 12                                           | 150                                   |  |
| Curve 4 0.6                                       | 52,700                                            | 20           | 41                  | 122                             | 249 ± 11                                           | 172                                   |  |
| Curve 5 0.44                                      | 54,600                                            | 14           | 30                  | 126                             | 232 ± 11                                           | 186                                   |  |

\* Note: Subsequent cooling from 250°C is air cooling.

TABLE IV

| Average Cooling Rate from 290 to 225°C, (°C/min.) | Tensile Properties                                |              |                     |                                 | Creep Tests at 20,000 lb/in. <sup>2</sup> at 68°F  |                                       |  |
|---------------------------------------------------|---------------------------------------------------|--------------|---------------------|---------------------------------|----------------------------------------------------|---------------------------------------|--|
|                                                   | Ultimate Tensile Strength (lb./in. <sup>2</sup> ) | % Elongation | % Reduction of Area | Hardness V.H.N. 5-Kilogram Load | Inverse Creep Rate ± 95% Confidence Limit (days/%) | Time to 1% Plastic Deformation (days) |  |
| 0.68                                              | 50,200                                            | 31           | 55                  | 112                             | 17.9 ± 1                                           | 8.7                                   |  |
| 0.33                                              | 47,500                                            | 31           | 56                  | 107                             | 28.0 ± 3.5                                         | 15                                    |  |

\* Note: Subsequent cooling from 225°C is air cooling.

TABLE V

| Method of Cooling from 250 to 50°C | Average Cooling Rate to Room Temperature (°C/min.) | Tensile Properties                                |              |                     |                                 |
|------------------------------------|----------------------------------------------------|---------------------------------------------------|--------------|---------------------|---------------------------------|
|                                    |                                                    | Ultimate Tensile Strength (lb./in. <sup>2</sup> ) | % Elongation | % Reduction of Area | Hardness V.H.N. 5-Kilogram Load |
| Ice water quenched                 | About 1400                                         | 56,100                                            | 17           | 25                  | 124                             |
| Air cooled                         | 19                                                 | 54,800                                            | 20           | 40                  | 124                             |
| Furnace cooled                     |                                                    |                                                   |              |                     |                                 |
| Curve 2                            | .22                                                | 45,800                                            | 23           | 50                  | 107                             |

TABLE VI

| Metallurgical Condition          | Tensile Properties                                |              |                     |
|----------------------------------|---------------------------------------------------|--------------|---------------------|
|                                  | Ultimate Tensile Strength (lb./in. <sup>2</sup> ) | % Elongation | % Reduction of Area |
| As heat treated                  | 52,500                                            | 29           | 45                  |
| After ageing for 10 days at 95°C | 51,300                                            | 17           | 35                  |

TABLE VII

| Alloy No. | Al   | Cu   | Alloy Composition, % | Heat Treatment              |                            | Tensile Properties                                |              |                     |    |
|-----------|------|------|----------------------|-----------------------------|----------------------------|---------------------------------------------------|--------------|---------------------|----|
|           |      |      |                      | Homogenizing Temperature °C | Air Cooling Temperature °C | Ultimate Tensile Strength (lb./in. <sup>2</sup> ) | % Elongation | % Reduction of Area |    |
| 36        | 25.5 | 0.98 | —                    | 380                         | R.T.                       | 38,200                                            | 40           | 70                  |    |
| 36        | 25.5 | 0.98 | —                    | 380                         | 250                        | 43,800                                            | 35           | 60                  |    |
| 40        | 25.5 | 3.34 | —                    | 380                         | R.T.                       | 40,800                                            | 28           | 48                  |    |
| 40        | 25.5 | 3.34 | —                    | 380                         | 250                        | 48,000                                            | 26           | 40                  |    |
| 83        | 25.7 | 1.03 | 0.055                | 380                         | R.T.                       | 45,800                                            | 22           | 50                  |    |
| 83        | 25.7 | 1.03 | 0.055                | 380                         | 250                        | 52,500                                            | 29           | 45                  |    |
| 52        | 22.1 | 2.75 | 0.059                | —                           | 380                        | R.T.                                              | 48,600       | 22                  | 30 |
| 52        | 22.1 | 2.75 | 0.059                | —                           | 380                        | 250                                               | 55,200       | 22                  | 30 |
| 79        | 26.3 | 5.1  | 0.06                 | —                           | 380                        | R.T.                                              | 50,300       | 20                  | 38 |
| 79        | 26.3 | 5.1  | 0.06                 | —                           | 380                        | 250                                               | 59,500       | 20                  | 30 |
| 80        | 24.9 | 10.2 | 0.05                 | —                           | 380                        | R.T.                                              | 56,500       | 11                  | 14 |

TABLE VII—Continued

## EFFECT OF THE TWO STAGE HEAT TREATMENT ON THE TENSILE PROPERTIES OF ALLOYS WITHIN THE SCOPE OF THE INVENTION

| Alloy | No.  | Al    | Cu    | Alloy Composition, % | Heat Treatment |     | Tensile Properties          |                            |                                                   |
|-------|------|-------|-------|----------------------|----------------|-----|-----------------------------|----------------------------|---------------------------------------------------|
|       |      |       |       |                      | Mg             | Bi  | Homogenizing Temperature °C | Air Cooling Temperature °C | Ultimate Tensile Strength (lb./in. <sup>2</sup> ) |
| 80    | 24.9 | 10.2  | 0.05  | —                    | 380            | —   | 250                         | 60,500                     | 9                                                 |
| 84    | 25.7 | 1.01  | 0.14  | 0.45                 | 380            | —   | R.T.                        | 49,400                     | 33                                                |
| 84    | 25.7 | 1.01  | 0.14  | 0.45                 | 380            | —   | 250                         | 58,000                     | 13                                                |
| 97    | 25.6 | —     | 0.134 | 0.53                 | 380            | —   | R.T.                        | 45,900                     | 26                                                |
| 84/85 | 93   | 22    | 1.00  | 0.136                | 0.44           | 380 | —                           | 250                        | 64,400                                            |
|       | 93   | 22    | 1.00  | 0.136                | 0.44           | 380 | —                           | R.T.                       | 46,900                                            |
|       | 94   | 31    | 1.02  | 0.140                | 0.46           | 380 | —                           | 250                        | 65,400                                            |
|       | 94   | 31    | 1.02  | 0.140                | 0.46           | 380 | —                           | R.T.                       | 49,300                                            |
|       | 49   | 12.78 | 0.80  | 0.022                | —              | 380 | —                           | 250                        | 69,200                                            |
|       | 49   | 12.78 | 0.80  | 0.022                | —              | 380 | —                           | R.T.                       | 42,100                                            |
|       | 49   | 12.78 | 0.80  | 0.022                | —              | 380 | —                           | 250                        | 56,800                                            |
|       | 49   | 12.78 | 0.80  | 0.022                | —              | 380 | —                           | 250                        | 21                                                |

We claim:

1. A heat treatment for improving the creep resistance of a wrought zinc-aluminum alloy having a zinc-aluminum eutectoid transformation, including a two-stage cooling process comprising:

- a. as the first stage of said process, slow cooling the alloy from above its eutectoid temperature and below its solidus or eutectic temperature to an intermediate temperature below the eutectoid temperature whereat the eutectoid transformation is substantially complete, and subsequently
- b. as the second stage of said process, upon attainment of said intermediate temperature, rapidly cooling said alloy to ambient temperature.

2. The heat treatment defined in claim 1 wherein said wrought alloy is a hot worked alloy.

3. The heat treatment defined in claim 1, wherein said intermediate temperature is at least 200°C.

4. The heat treatment defined in claim 1 wherein said alloy is homogenized at a temperature above its eutectoid temperature and below its solidus or eutectic temperature before the commencement of said slow cooling.

5. The heat treatment as defined in claim 4 wherein said slow cooling of the alloy is effected by allowing a furnace used for said heat treatment to cool at its natural rate.

6. The heat treatment as defined in claim 4 wherein said rapid cooling of said alloy is effected by air cooling the alloy.

7. The heat treatment as defined in claim 4 wherein said slow cooling is at an average rate of less than about 2.0°C./min. to the temperature at which said rapid cooling commences.

8. The heat treatment as defined in claim 4 wherein slow cooling comprises cooling said alloy from above its eutectoid temperature and below its solidus temperature to a temperature of 250°C. at an average rate of less than about 2°C./min.

9. The heat treatment as defined in claim 4 wherein the rapid cooling is commenced at about 250°C.

10. The heat treatment for improving the creep resistance of a wrought zinc-aluminum alloy containing 12 to 30% aluminum, 0 to 10% copper, 0 to 1% magnesium, 0 to 3% bismuth, the balance being zinc except

for incidental impurities, including a two stage cooling process comprising:

a. as the first stage of said process, homogenizing and slow cooling the alloy from above its eutectoid temperature and below its solidus or eutectic temperature to an intermediate temperature below its eutectoid temperature whereat the eutectoid transformation is substantially complete, and subsequently

b. as the second stage of said process, upon attainment of said intermediate temperature, rapidly cooling said alloy to ambient temperature.

11. A heat treatment for improving the creep resistance of a wrought zinc-aluminum alloy containing 18 to 30% aluminum, 0 to 10% copper, 0 to 1% magnesium, 0 to 3% bismuth, the balance being zinc except for incidental impurities, including a two-stage cooling process comprising:

a. as the first stage of said process homogenizing and slow cooling the alloy from above its eutectoid temperature and below its solidus temperature to an intermediate temperature below its eutectoid temperature whereat the eutectoid transformation is substantially complete, and subsequently

b. as the second stage of said process, upon attainment of said intermediate temperature, rapidly cooling said alloy to ambient temperature.

12. The heat treatment as defined in claim 11 wherein said alloy is homogenized at a temperature such that said alloy is substantially in the  $\alpha'$  phase.

13. The heat treatment defined in claim 11 wherein said wrought alloy is a hot worked alloy.

14. A heat treatment for improving the creep resistance of wrought zinc-aluminum alloys containing 18 to 30% aluminum, 0 to 10% copper, 0 to 1% magnesium, 0 to 3% bismuth, the balance being zinc except for incidental impurities, said treatment including a two-stage cooling process comprising:

a. as the first stage of said process, homogenizing the alloy at about 380°C., and slow cooling the alloy from the homogenization temperature to an intermediate temperature of about 250°C. at an average rate of cooling of about 1°C./min. and subsequently

b. as the second stage of said process, upon attainment of said intermediate temperature, air cooling said alloy from about 250°C. to ambient temperature.

\* \* \* \* \*